

Oct. 22, 1974

W. KELLER ET AL

**3,843,331**

APPARATUS FOR PRODUCING A RADIALLY UNIFORM RESISTANCE  
CHARACTERISTIC IN A SEMICONDUCTOR CRYSTAL BY USE  
OF HIGH FREQUENCY SONIC VIBRATIONS

Filed Dec. 1, 1972

### 3. Sheets-Sheet 1



Fig.1



Fig.2



Fig. 3

Oct. 22, 1974

W. KELLER ET AL

3,843,331

APPARATUS FOR PRODUCING A RADIALLY UNIFORM RESISTANCE  
CHARACTERISTIC IN A SEMICONDUCTOR CRYSTAL BY USE  
OF HIGH FREQUENCY SONIC VIBRATIONS

Filed Dec. 1, 1972

3 Sheets-Sheet 2

Fig.4



Oct. 22, 1974

W. KELLER ET AL

3,843,331

APPARATUS FOR PRODUCING A RADIALLY UNIFORM RESISTANCE  
CHARACTERISTIC IN A SEMICONDUCTOR CRYSTAL BY USE  
OF HIGH FREQUENCY SONIC VIBRATIONS

Filed Dec. 1, 1972

3 Sheets-Sheet 3

Fig.5



## 1

3,843,331

### APPARATUS FOR PRODUCING A RADIALLY UNIFORM RESISTANCE CHARACTERISTIC IN A SEMICONDUCTOR CRYSTAL BY USE OF HIGH FREQUENCY SONIC VIBRATIONS

Wolfgang Keller, Walter Lugscheider, and Alfred Muehlbauer, Munich, Germany, assignors to Siemens Aktiengesellschaft, Berlin and Munich, Germany  
Continuation-in-part of application Ser. No. 283,320, Aug. 24, 1972. This application Dec. 1, 1972, Ser. No. 311,380

Claims priority, application Germany, Dec. 2, 1971,  
P 21 59 916.6  
Int. Cl. B01j 17/00

U.S. CL. 23—301 SP

15 Claims

#### ABSTRACT OF THE DISCLOSURE

A method and apparatus for producing a radially uniform resistance characteristic in a semiconductor single crystal rod by subjecting a stock polycrystalline semiconductor rod to a floating melt zone purification and substantially simultaneously charging the stock rod with sonic oscillations in the rod axial direction. The sonic oscillations are generated by an electromechanical sound generator means, such as a piezoelectric sound generator means or a magnetostrictive sound generator means, at a frequency greater than 20 kHz. The sound generator means is mounted directly on a rod holding means and the high frequency sonic oscillations are transmitted to the melt zone of the rod by a coupling medium, such as composed of a lead-tin alloy or a tetrafluoroethylene-epoxy resin, positioned between one end of the rod and adjacent rod mounting means. In certain embodiments, the electromechanical sound generator means is positioned at an angle to the rod axis so that the sonic oscillations travel in a direction forming a select angle up to 10° with the axis.

#### CROSS-REFERENCE TO RELATED APPLICATION

This is a continuation-in-part application of my copending application U.S. Ser. No. 283,320, filed Aug. 24, 1972.

#### BACKGROUND OF THE INVENTION

##### Field of the Invention

The invention relates to production of semiconductor crystals and more particularly to a method and apparatus for producing a radially uniform resistance characteristic in a monocrystalline semiconductor rod.

##### Prior Art

The production of monocrystalline semiconductor rods by floating melt zone techniques is known. Generally, polycrystalline semiconductor rods, such as of silicon, are transformed into single or monocrystalline structures by placing a seed crystal at one end of the polycrystalline stock rod and establishing an annular melt zone at such end and then slowly moving the melt zone along the rod to the other end thereof. The re-solidified portion attains a higher degree of crystalline order and forms a single crystal. In such arrangements, the semiconductor rod is generally vertically mounted between a pair of movable mounting means, one of which rotates about the axis of the rod during the movement of the melt zone so as to assure a symmetrical growth of the re-solidified portion.

Single crystal rods produced by floating melt zone techniques exhibit a radially variable resistance characteristic, apparently because of insufficient mixing within the melt zone thereof. Of course, it is highly desirable in the production of semiconductor components that the semiconductor substrate have a radially uniform resistance characteristic.

## 2

My earlier application U.S. Ser. No. 283,320 discloses a novel means of achieving improved mixing within a melt zone. The principles of that invention were demonstrated by charging an unmixed dye solution with sonic oscillations to achieve a substantially homogeneous solution. 5 The application discloses that a good mixing within a melt zone can be achieved across a rod cross-section by charging at least one rod mounting means with audio sonic oscillations in the rod axial direction during the floating melt zone purification process. Rods treated in this manner exhibit a much more uniform radial resistance characteristic than conventionally produced semiconductor rods which have undergone a floating melt zone purification. Nevertheless, it is desirable to achieve an 10 improved radially uniform resistance characteristic.

#### SUMMARY OF THE INVENTION

The invention provides a novel method and apparatus for producing a monocrystalline semiconductor rod characterized by a radially uniform resistance characteristic.

It is a novel feature of the invention to electrically generate sonic oscillations at a frequency greater than 20 kHz. by means of electromechanical sound generator means and to transfer such high frequency sonic oscillations to the melt zone of a semiconductor crystal rod having a floating melt zone via a coupling medium positioned between the stock rod and a rod mounting means.

It is a further novel feature of the invention to interconnect the melt zone of a semiconductor crystal rod with a cooled piezoelectric sound generator means or with a cooled magnetostrictive sound generator means via a rigid or muffling coupling medium.

It is another novel feature of the invention to position a sound generator means on a rod mounting means in such a manner that the generator sonic oscillations radiate in a direction that forms a select angle with the semiconductor rod axis. In one embodiment, this angle is adjustable up to a maximum of 10° from the rod axis and in another embodiment up to a maximum of 1° from the rod axis. In a further embodiment, the sound generator is positioned to emit sonic waves in a direction that forms an angle to the rotational axis of the semiconductor crystal rod and the semiconductor crystal rod is mounted to rotationally eccentric movement.

It is yet another novel feature of the invention to regulate the amplitude of sonic oscillations charged to the melt zone of a semiconductor crystal rod having a floating melt zone to a constant value as the melt zone moves along the rod by measuring the amplitude of modulation of the heating frequency (utilized to establish the melt zone) through the sonic oscillations.

#### BRIEF DESCRIPTION OF THE DRAWINGS

FIG. 1 is a partial elevated sectional view of a semiconductor crystal rod being treated in accordance with the principles of the invention;

FIG. 2 is a partial sectional view of an embodiment constructed in accordance with the principles of the invention;

FIG. 3 is a similar view of another embodiment constructed in accordance with the principles of the invention;

FIG. 4 is a schematic illustration of a circuit utilized in accordance with the principles of the invention for maintaining the amplitude of sonic oscillations at a constant level within the floating melt zone; and

FIG. 5 is a schematic representation of a component of the circuit illustrated at FIG. 4.

#### DESCRIPTION OF THE PREFERRED EMBODIMENTS

The invention provides a means of producing semiconductor crystal rods having a radially uniform resist-

ance characteristic which is relatively simple, capable of yielding reproducible results and producing high quality semiconductor crystal rods.

Generally, the invention comprises subjecting a stock semiconductor crystal rod to a floating melt zone purification and subjecting the melt zone to axially directed high frequency sonic oscillations. In this manner, extremely good mixing action of the melt is always assured. The matter within the melt zone is homogeneously distributed throughout the zone so that upon solidification thereof, a uniform or substantially uniform radial resistance characteristic through a cross-section of such a crystal is attained.

Substantially all semiconductor materials can be subjected to the beneficial processing of the invention. Silicon is an extremely common semiconductor material and a stock crystal thereof is readily processed in accordance with the invention to attain radially uniform resistance characteristics.

In accordance with the principles of the invention, sonic oscillations are electrically generated through an electro-mechanical sound generator at a frequency of more than 20 kHz, and transferred to a crystal rod via a rigid or flexible coupling medium positioned between the rod and a rod mounting means.

Preferred electromechanical sound generator means include cooled magnetostrictive sound generator means and cooled piezoelectric sound generator means that produce longitudinal sound waves in the semiconductive crystal rod being processed. Such electromechanical sound generator means produce a higher crystal order within zone-melted single crystal rods in comparison to the crystal order achieved by my earlier described invention. Density fluctuations due to crystalline imperfections that cause viscosity fluctuations during crystalline growth processes are decreased; also gas bubbles, gas bubble agglomerates, density fluctuations, such as vacant lattice sites (Schottky and/or Frenkel defects) resulting from crystal growth, vacant lattice site agglomerations, doping in-homogeneities, which are sometimes referred to as "striations," etc. are decreased in the solidified matter. The mixing of the molten material is considerably favored in the proximity of the solidification front by the radiation of sound waves. Accordingly, the radiation of sound waves can occur from a seed crystal or via the stock rod.

In a preferred embodiment, the electromechanical sound generator means is positioned on a rod mounting means so that the direction of sound waves produced thereby forms an angle with the rod axis. Preferably, this angle is adjustable up to a maximum of about 10° from the rod axis. With such an arrangement of an electromechanical sound generator means, additional mixing effects are created because of the transversal components in the sound waves.

The select electromechanical sound generator means is suitably energized via means, such as an electrical circuit, to produce sonic oscillations having a frequency in the range of 20 kHz. to 10 mHz. The select sonic frequency may be continuously or irregularly varied in the region of sound amplitude in an amount approximately greater than the period of density fluctuation  $D_{D1}$  and  $D_{D2}$  (FIG. 1), wherein  $D_1$  is the period of coarse striations and  $D_2$  is the period of fine striations. By correctly applying sound radiations of 10 to 1000 w./cm.<sup>2</sup> (watts per centimeter squared), sonic frequencies are produced that are in the kilohertz (kHz.) to megahertz (mHz.) range. The vibration amplitude  $A$  is proportional to the dimension  $D$ , defined by the period of coarse striations  $D_{D1}$ , fine striations  $D_{D2}$  and the melt zone length  $D_z$ . The amplitude  $A$  of the vibrations is in all instances determined by the radiation power of a select fixed frequency in accordance with the equation:

$$\frac{A}{\lambda} = \sqrt{\frac{J}{(2\pi^2)(\rho)(C_1^3)}} \quad (I)$$

wherein:

$J$  is the work in w./m.<sup>2</sup> (watts per square meter);  
 $\rho$  is the specific weight in t./m.<sup>3</sup> (unit mass per cubic meter);

5  $C_1$  is the speed in m./s. (meters per second); and  
 $\lambda$  is the sonic wavelength

and provide the following results:

|    | $J$                         | $A$                   | $f$         |
|----|-----------------------------|-----------------------|-------------|
| 10 | 100, w./cm. <sup>2</sup>    | 20 $\mu\text{m.}$     | 65 kHz.     |
|    | 100, w./cm. <sup>2</sup>    | 200 $\mu\text{m.}$    | 6.5 kHz.    |
|    | 10-100, w./cm. <sup>2</sup> | 20-200 $\mu\text{m.}$ | =5-100 kHz. |

15 These conditions are more readily visualized by considering FIG. 1. A stock polycrystalline semiconductor rod 1, such as composed of silicon, undergoing a floating melt zone purification process is illustrated. Of course, such a stock rod 1 is positioned in a melt zone purification apparatus (not shown) which typically includes a housing connected to a vacuum pump so that the interior chamber thereof is evacuated, a pair of movable mounting means extending from opposing walls thereof for supporting the stock rod therebetween, a heating means, such as an induction coil that encompasses a portion of the rod and defines a melt zone thereon, suitable energy sources and circuitry for transmitting the same, means for selectively moving the rod within the housing, etc. For the sake of brevity, most of such conventional structure has been omitted 20 from the drawings and will be generally referred to in the specification and claims as a floating melt zone operational environment FMZ.

25 Referring back to FIG. 1, the solidified monocrystalline rod portion is designated by reference numeral 2; reference numeral 3 designates a melt zone located between the rod mounting means (not shown) and reference numeral 4 designates an induction heating coil which provides a requisite heat to produce the melt zone. Reference numeral 5 designates a sound generator means producing longitudinally radiating sound waves in the direction of arrow 5a, which is generally parallel with the rod axis.

30 The symbol  $D_z$  indicates the approximate melt zone length, generally about 15 to 30 mm. (millimeters), the symbol  $D_D$  refers to the period of density fluctuation 35 wherein the coarse form of striations  $D_{D1}$  are about 100 to 200  $\mu\text{m.}$  (micrometers) and the fine form of striations  $D_{D2}$  are about 5 to 20  $\mu\text{m.}$  The requisite sonic power for effecting such density fluctuations is readily determined by 40 the above formula (I).

45 In an embodiment of the invention, the amplitude of sonic oscillations charged to the rod axis is regulated in relation to the position of the melt zone on the rod so as to be at a constant value within the melt zone. The sonic amplitude is regulated by measuring the amplitude of 50 modulation of the induction coil heating frequency through the sonic oscillations. In this manner, a certain degree of independence between the sonic oscillations charged to the rod and the location of the melt zone on the rod is 55 achieved.

60 In exemplary embodiments, the coupling medium between the semiconductor rod and the rod mounting means is selected from the group consisting of rigid and dampening or muffling mediums. Rigid mediums are preferably composed of metal and metal alloys, such as lead-tin alloys and the muffling mediums are preferably composed of an inorganic putty or plastic material, such as an epoxy resin modified with polytetrafluoroethylene (Teflon—a registered trademark).

65 The coupling medium must interconnect the rod mounting means with the rod over a uniformly large area in order to avoid high sonic power densities. The elastic characteristic of the coupling medium determines the amount of dampening and the phase location of the sonic waves entering the melt zone.

Crystals treated in accordance with the principles of the invention need no further treatment to achieve crystal order perfection. Doping material included during the growth of a crystal (radially non-homogeneously) is redistributed in a radially homogeneous manner. Components produced from such crystal rods have a higher quality due to the more homogeneous starting materials as compared with crystals subjected to more conventional dopant diffusion. For example, higher blocking voltages are more readily attained in semiconductor crystals treated in accordance with the principles of the invention, which are necessary for silicon raster vidicon structures.

Referring now to FIG. 2 wherein an upper portion of a stock rod 10 in a floating melt zone operational environment FMZ<sub>o</sub> is shown. The stock rod 10 is composed of polycrystalline silicon and is mounted at its upper portion in a rod mounting means 11. A coupling medium 12, here shown as being composed of a plastic material, is positioned between the upper end of rod 10 and the adjacent surface of the mounting means 11. In preferred apparatus embodiments of the invention, the rod mounting means 11 is mounted in a vacuum-tight and selectively movable manner on a wall of floating melt zone housing. Such mountings are conventional and thus not shown. A sound generator means 13, which may be a water-cooled piezoelectric sound generator means or a water-cooled magnetostrictive sound generator means is positioned above the mounting means 11 and in direct contact therewith. In order to increase the mixing action within the melt zone (not shown) and thereby diminish dopant fluctuations within the produced single crystal rod, the rod mounting means 11 is connected with the sound generator means 13 in such a manner that the sound waves are radiated at an angle 17, up to a maximum of 10° to the rod axis 18. The angle 17 is adjustable, for example, by varying the angles that the upper surface 11a of the mounting means 11 forms with the lower surface 11b thereof. The thus created transversal sound waves cause an additional stirring or mixing effect within the melt zone. A mounting means 14 supports the sound generator means 13 and may be rotationally driven by a power source (not shown) outside of the floating melt zone housing.

FIG. 3 illustrates another embodiment of the invention and portions thereof similar to portions in FIG. 2 have the same reference numerals. In this embodiment, the coupling media 12a is composed of a metal and the rod mounting means 11 is provided with an upper surface 11a which forms a smaller angle with the lower surface 11b thereof so that the sound waves generated by the sound generator means 13 radiate in a direction S that forms an angle 17 up to a maximum of 1° with the rod axis 18. Of course, angle 17 is adjustable. The mounting means 14 may be attached to a suitable drive means (not shown) to rotate the rod 10 in an eccentric or wobbling movement to achieve further mixing action within the melt zone.

FIG. 4 illustrates an operational circuit for maintaining the amplitude of sonic oscillations at a constant level within a floating melt zone by measuring the amplitude of modulation of a heating frequency through the sonic oscillations. An induction heating coil 4 surrounds a portion of a semiconductor rod 10 so as to define a melt zone D<sub>z</sub> thereon. A tuning capacitor 26 is positioned within the heating circuit supplying energy to the induction coil 4. The heating circuit includes a high frequency generator means 22, a decoupling coil 21 and a demodulator means which include a demodulator diode 23 and an electronic filter 24 for separating the ultrasonic modulation signal from the rectified high frequency signal. An amplifier 25 receives the signal from the filter 24 and transmits it to a desired actual-value comparison stage 26. A reference signal source 29 feeds an appropriate signal into stage 26 and stage 26 then feeds another appropriate signal to controlling stage 27, which controls

an ultrasonic power supply 28. The power supply 28 transmits the required electrical energy to an electromechanical sound generator means 13 to produce the desired sonic oscillations.

FIG. 5 illustrates in some detail the circuitry of the desired actual-value comparison stage 26 as well as its interconnection with other related components in the circuit shown at FIG. 4. The stage 26 comprises a difference amplifier that is formed by two tubes 41 and 42 and a common cathode resistance 43, which is grounded. A polarized relay 44 is located in the anode branch of this circuit. The anode voltage is symmetrically guided to the tubes 41 and 42 via a coil 45 of the polarized relay 44. The relay 44 includes a set of transfer contacts which include stationary contacts 46 and 47 and a moving arm 48.

A desired signal is transmitted to the grid of tube 42 from the reference signal source 26 wherein the desired signal is produced by an adjustable potentiometer 50 and a voltage source 49. The reference signal source is grounded to the difference amplifier of stage 26 at the side opposite that connected to the grid of tube 42. The grid of the other tube 41 receives the actual signal from the amplifier 25. Depending in which direction the actual signal deviates from the desired signal, either tube 41 or tube 42 directs current through the coil 45 of the relay 44 so that the switching arm 48 is moved either to contact 46 or 47.

In the controlling stage 27, two motors 52 and 53 are coupled by the contacts 46 and 47 respectively to an alternating current source 51, which supplies alternating electrical current to the motors. The motors 52 and/or 53 readjust the ultrasonic current supply 28 to correspond to the deviation of the actual signal from the desired signal in such a manner that the energy supplied by the ultrasonic current supply 28 corresponds to the desired signal.

As is apparent from the foregoing specification, the present invention is susceptible of being embodied with various alterations and modifications which may differ particularly from those that have been described in the preceding specification and description. For example, the angle 17 may be adjusted by varying the relation of other surfaces, such as of the coupling media or of the sound generator means to the crystal rod axis, to achieve the select angle between the sound wave direction and the crystal rod axis. For this reason, it is to be fully understood that all of the foregoing is intended to be merely illustrative and is not to be construed or interpreted as being restrictive or otherwise limiting of the present invention, excepting as is set forth and defined in the here-to-appendant claims.

We claim as our invention:

1. In a method of producing a radially uniform resistance characteristic in a semiconductor crystal rod that includes positioning the semiconductor rod in a floating melt zone operational environment and subjecting said rod to axially directed sonic oscillations, the improvement comprising, electrically generating said sonic oscillations at a frequency higher than 20 kHz. by an electromechanical sound generator means and transferring said sonic oscillations to said rod.
2. A method as defined in claim 1 wherein said sonic oscillations are generated at a frequency in the range of 20 kHz. to 10 mHz.
3. In a method as defined in claim 1 wherein said sonic oscillations are radiated in a direction which forms an angle with the axis of said rod.
4. In a method as defined in claim 1 wherein said sonic oscillations are radiated in a direction which forms a select angle up to 1° with the axis of said rod.
5. In a method as defined in claim 1 wherein said sonic oscillations are radiated in a direction which forms a select angle up to 10° with the axis of said rod.
6. In a method as defined in claim 1 wherein said sonic oscillations are radiated in a direction which forms an

angle with the axis of said rod and said rod is rotated through an eccentric path of travel.

7. In a method as defined in claim 1 wherein the amplitude of sonic oscillations is regulated in relation to the location of the melt zone on said rod so as to maintain a constant value therein by measuring the amplitude of modulation of a heating frequency utilized to establish said melt zone through the sonic frequencies.

8. An apparatus for producing a radially uniform resistance characteristic in a semiconductor crystal rod comprising: an operational environment for a floating melt zone purification process including a pair of opposing crystal rod mounting means and an induction heating coil encompassing a portion of said rod to define a melt zone therein; an electrically energized electromechanical sound generator means capable of producing sonic oscillations with a frequency over 20 kHz, positioned outside said operational environment; a coupling medium connected at one end thereof to said electromechanical sound generator means and at the other end thereof to one of said pair of rod mounting means for transmitting said sonic oscillations to said rod, and means for energizing said electromechanical sound generator means.

9. An apparatus as defined in claim 8 wherein said electromechanical sound generator means comprises a cooled piezoelectric sound generator means.

10. An apparatus as defined in claim 8 wherein said electromechanical sound generator means comprises a cooled magnetostrictive sound generator means.

11. An apparatus as defined in claim 8 wherein said coupling medium is composed of a material selected from the group consisting of rigid and muffling mediums.

12. An apparatus as defined in claim 11 wherein said coupling medium is composed of a material selected from the group consisting of metals, metal alloys and plastics.

13. In an apparatus for producing a radially uniform resistance characteristic in a semiconductor crystal rod, which includes an operational environment for a floating melt zone process having a pair of opposing crystal rod mounting means, each of said mounting means having an

upper and lower surface, the improvement comprising: a coupling medium capable of transmitting sonic oscillations positioned in direct contact with an upper surface of said rod and a lower surface of one of said rod mounting means, an electromechanical sound generator means capable of producing longitudinal sonic oscillations at a frequency in the range of 20 kHz. to 10 mHz. positioned in direct contact with an upper surface of said one of said rod mounting means and means for energizing said electromechanical sound generator means.

14. In an apparatus as defined in claim 13 wherein said one of said rod mounting means is provided with an upper surface thereof that forms an angle with the lower surface thereof whereby said sonic oscillations generated by said sound generator means in contact with such upper surface radiate in a direction that forms an angle with the axis of said crystal rod.

15. In an apparatus as defined in claim 14 including a means for moving said rod in a rotationally eccentric path of travel.

#### References Cited

#### UNITED STATES PATENTS

|           |         |         |       |           |
|-----------|---------|---------|-------|-----------|
| 3,206,286 | 9/1965  | Bennett | ----- | 23—273 SP |
| 3,216,805 | 11/1965 | Emeis   | ----- | 23—273 SP |
| 2,952,722 | 9/1960  | Jackson | ----- | 23—273 SP |
| 3,543,531 | 12/1970 | Adams   | ----- | 23—273 SP |
| 3,340,016 | 9/1967  | Wirth   | ----- | 23—273 SP |
| 3,637,439 | 1/1972  | De Bie  | ----- | 23—273 SP |
| 3,592,937 | 7/1971  | Emeis   | ----- | 23—273 SP |
| 3,716,341 | 2/1973  | Schmidt | ----- | 23—273 SP |
| 3,655,345 | 4/1972  | Longo   | ----- | 23—301 SP |
| 3,615,245 | 10/1971 | Emeis   | ----- | 23—301 SP |

NORMAN YUDKOFF, Primary Examiner

F. SEVER, Assistant Examiner

U.S. CL. X.R.

40 23—273 SP